

# United States Patent

[11] 3,623,987

|                |                                                                                                                   |                                                |
|----------------|-------------------------------------------------------------------------------------------------------------------|------------------------------------------------|
| [72] Inventors | Robert Alan Cameron Ker;<br>Robert Carswell; John Lavington Clarke;<br>Peter Anthony Burt, all of London, England | 2,916,457 10/1959 Friedrich et al. .... 252/75 |
| [21] Appl. No. | 3,553                                                                                                             | 3,218,256 11/1965 Edwards et al. .... 252/47.5 |
| [22] Filed     | Jan. 8, 1970                                                                                                      | 3,274,113 9/1966 Reiland ..... 252/78          |
| [45] Patented  | Nov. 30, 1971                                                                                                     | 2,629,693 2/1953 Barton et al. .... 252/33.4   |
| [73] Assignee  | Costrol Limited<br>London, England                                                                                | 2,542,785 2/1951 Walker ..... 252/79           |

[32] Priority June 18, 1964  
[33] Great Britain  
[31] 25,326/64

[54] **FUNCTIONAL FLUIDS**  
19 Claims, No Drawings

[52] U.S. Cl. .... 252/79,  
252/56, 252/77, 252/79  
[51] Int. Cl. .... C09k 3/02  
[50] Field of Search. .... 252/56, 73,  
75, 76, 79; 260/485 G

[56] **References Cited**

UNITED STATES PATENTS  
2,857,421 10/1958 Matuezak et al. .... 260/485

Primary Examiner—Leon D. Rosdol  
Assistant Examiner—P. E. Willis

**ABSTRACT:** This invention is for improvements in or relating to hydraulic fluids and is particularly concerned with liquids employed as the power-transmitting medium in hydraulic brake systems for vehicles, for example, motor cars and airplanes. The hydraulic fluid of the invention contains at least 50 percent by weight of at least one ester of the formula



wherein R is an alkylene group of from two to eight carbon atoms, R<sup>1</sup> is an alkyl of from one to six carbon atoms or a phenyl radical, R<sup>2</sup> is ethylene, propylene or butylene and n is an integer of from zero to three.

## FUNCTIONAL FLUIDS

This is a continuation of a application Ser. No. 464,211 filed June 15, 1965, now abandoned

## BACKGROUND OF THE INVENTION

Hydraulic brake systems comprise metal and rubber parts which are exposed to the liquid employed as the power transmitting medium and it is essential that a liquid be used which has little, if any attack on either the metal or the rubber parts of the brake system, either at ordinary temperatures or at the elevated temperatures which are setup in the parts of the system adjacent to the braking surfaces during a prolonged application of the brakes. It is further more essential that the hydraulic transmission medium should be stable and of a high boiling point such as not to vaporize to any substantial extent under operating conditions. Again, the liquid should have a low freezing point to withstand operating temperatures which obtain either during cold weather, or in the case of aircraft, during high altitude flight. In addition it is necessary that the liquid shall have a sufficiently low viscosity to render the system readily operable, the viscosity not changing to any material extend under operating conditions. Finally further important considerations are that the liquid shall have a low rate of vaporization and also sufficient lubricating properties properly to lubricate the moving parts of the system.

In the hydraulic systems of motor cars typical "heavy duty" brake fluids in service at the present time boil at about 216°C. With the generally increasing severity of operation, however, especially in vehicles fitted with disc brakes, there is a need for hydraulic fluids having even higher boiling points and fluids boiling at about 260°C. are now being called for. Fluids of this latter type in commercial use normally comprise a major proportion of one or more polyethylene glycols, ethers or polyethylene glycols, or mixtures of such compounds. Minor proportions of castor oil or lubricity additives, such as polyalkylene glycol polyesters, may be present, together with one or more corrosion inhibitors.

In practice, it is found that hydraulic brake fluids based on polyethylene glycols and/or ethers thereof, are hygroscopic and in process of time water is absorbed from the atmosphere and the boiling point steadily falls. Thus, after a period of use, two brake fluids having initial boiling points more than 56°C. apart may be found to have boiling points of the same order, both substantially below the initial boiling points of the fluids. It is not uncommon, for example, for a brake fluid, after several months service, to be found to contain about 1 percent of water and, on prolonged service, up to 3 percent of water may be found in such fluids.

In a simple laboratory experiment, a typical known hydraulic brake fluid, fluid A, having an initial boiling point of 216°C., was found to have a boiling point of 182°C. when 1 percent of water was added and a boiling point of only 141°C. when 3 percent of water was present. A known high-temperature brake fluid, fluid B, which had an initial boiling point of 271°C. was found to have a boiling point of 204°C. when 1 percent of water was present and of only 154°C. when 3 percent of water was present. The high temperature brake fluid, therefore, had become inferior to the conventional brake fluid in its original condition as a result of absorbing only 1 percent of water.

In another simple laboratory test in which 150 mls. of fluid were placed in open 250 ml. beakers and exposed to the atmosphere of the laboratory, it was found that the boiling point of the conventional brake fluid, Fluid A, fell from 216°C. to 137°C. in 4 days, whereas the boiling point of the high-temperature brake fluid, fluid B, fell from 271°C. to 146°C. in 4 days. The advantage of fluid B over fluid A was thus dissipated in a very short time.

It is important for a hydraulic brake fluid to retain a high boiling point throughout its useful life since a reduction in boiling point may result in the formation of vapor locks with consequent failure of the braking system. In order to avoid this possibility, it is necessary for current high-temperature brake

fluids based on polyglycols and/or polyglycol ethers, to be changed fairly frequently in the braking system, so that moisture is not allowed to accumulate. It is desirable that the boiling point of a fluid should not be allowed to fall below about 149°C.

We have found that high-temperature hydraulic fluids, which have relatively low hygroscopicity and high boiling points, may be formulated from certain esters of organic dicarboxylic acids and ethers of certain glycols.

10 The invention provides a hydraulic fluid having a kinematic viscosity at -40°C. of not more than 5,000 centistokes, preferably not more than 2,000 centistokes, and preferably having a boiling point of at least 260°C., and either consisting of or comprising at least 50 percent by weight, preferably at least 80 percent of at least one ester having the general formula



where R is a straight or branched chain alkylene group which contains at least two, preferably from two to eight carbon atoms, R<sup>1</sup> is an alkyl radical having from one to four preferably one to two carbon atoms or a phenyl radical R<sup>2</sup> is ethylene, propylene or butylene group, and n is 0, 1 2 or 3, together with a minor amount of at least one additive. The groups R<sup>1</sup>, R<sup>2</sup> and n may be the same or different.

Preferred acids R(COOH)<sub>2</sub> from which the esters are derived are succinic, glutaric, adipic, azelaic, sebacic and isosebacic acids, although other dicarboxylic acids may be used, if desired, e.g. a commercially available mixture of adipic, glutaric and succinic acids, known as "A.G.S. acid." Preferred examples of the glycol ethers from which the esters are made are:

Ethylene glycol monomethyl ether ("Methyl Oxitol" or "Methyl Cellosolve").

40 Diethylene glycol monoethyl ether ("Dioxitol" or "Carbitol").

Diethylene glycol monomethyl ether ("Methyl Dioxitol" or "Methyl Carbitol").

45 Triethylene glycol monomethyl ether ("Methyl Trioxitol").

Ethylene glycol monoethyl ether ("Ethyl Oxitol").

Triethylene glycol monoethyl ether ("Ethyl Trioxitol").

Preferred esters in accordance with the present invention are given in table I together with their physical properties, it being understood that when the esters have too high a viscosity, particularly at -40°C., then they may be blended with a suitable ester or a small amount of inert diluent to give a fluid having the viscosity requirements in accordance with the present invention. For example a blend of 15 percent di(ethyl trioxitol) sebacate and 85 percent (methyl oxitol adipate had the following viscosity characteristics:

1,006 cS. @ -40°C.

8.76 cS. @ cS. c80140 38°C.

2.63 cS. @ 99°C.

60 Typical additives which may be used in the invention are lubricity additives selected from castor oil or castor oil treated in various ways, for example,

Firsts Castor oil,

Castor oil to specification DTD72

Blown castor oil, i.e. castor oil blown with air or oxygen while being heated.

Special Pale Blown Castor i.e. a similarly blown castor.

"Hydrin 4" i.e. a commercially available ethylene/oxide/propylene oxide treated castor oil.

70 Other lubricity additives which may be incorporated in hydraulic fluids in accordance with the present invention include borate esters e.g. tricresyl borate and phosphorus-containing esters, especially phosphates e.g. tricresyl phosphate.

The hydraulic fluids of the present invention may also include minor proportions of polyalkylene or ethers thereof

e.g. those sold under the Reg. Trade Mark "Ucon", particularly those of the LB and HB series. Suitable examples of these polyoxyalkylene glycols and their ethers and esters are given in our copending application No. 337,181 filed Jan. 13, 1964 now U.S. Pat. No. 3,334,048 together with examples of other suitable lubricity agents, such as orthophosphate or sulfate salts of primary or secondary aromatic amines, dialkyl citrates, aliphatic dicarboxylic acids and esters thereof, specific examples being

Diamylamine orthophosphate  
 Dinonylamine orthophosphate  
 Diamylamine sulphate  
 Dinonyl citrate  
 Di (2-ethyl hexyl) citrate  
 15 Polyoxyethylene sebacate derived from a polyoxyethylene glycol of M.W. 200  
 Polyoxyethylene azelate derived from polyoxyethylene glycol of M.W. 200  
 20 Polyoxyethylene polyoxypropylene glutarate derived from mixed polyoxyglycols of average M.W. of about 200  
 Glutaric acid  
 Axelaic acid  
 Sebacic acid  
 Succinic acid  
 Di ethyl sebacate  
 Di 2-ethyl hexyl sebacate  
 Di iso octyl azelate  
 Unsaturated aliphatic acids or their salts may also be used e.g. oleic acid or potassium ricinoleate.

Corrosion inhibitors which may be used in the present invention may be selected from heterocyclic nitrogen-containing compounds e.g. benzotriazole and benzotriazole derivatives such as those described in British Pat. specification No. 1,061904 or mercapto benzothiazole. Many amines or derivatives thereof are also suitable as corrosion inhibitors, for example

di n-butylamine  
 di n-aminolamine  
 cyclohexylamine  
 morpholine  
 triethanolamine  
 and soluble salts thereof e.g. cyclohexylamine carbonate.  
 Phosphites are also good corrosion inhibitors e.g.  
 Tri phenyl phosphite  
 Di isopropyl phosphite  
 and certain inorganic salts may be incorporated e.g. sodium nitrate.

Other additives which may be included are antioxidants such as diarylamines e.g. diphenylamine, p,p'-diocetyl diphenylamine, phenyl- $\alpha$ -naphthylamine or phenyl- $\beta$ -naphthylamine. Other suitable antioxidants are those commonly known as hindered phenols which are exemplified by 2,4dimethyl-6-t-butyl phenol  
 2,6 di-t-butyl -4-methyl phenol  
 2,6 di-t-butyl phenol  
 1,1 bis(3 5 di-t-butyl-4-hydroxyphenyl)methane  
 3,3',5,5' tetra-t-butyl-4-4'-dihydroxydiphenyl  
 3-methyl 4,6di-t-butyl phenol  
 4-methyl-2-t-butyl phenol

Yet further additives which may be used are phenothiazine and its derivatives, for example those having alkyl or aryl, groups attached to the nitrogen atom or to the aryl groups of the molecule.

These additives will normally be employed in conventional amounts which, in many cases, will be from 0.05 percent to 10 percent, for example from 0.1 percent to 2 percent by weight.

In formulating brake fluid compositions to meet the requirements of SAE 70R3 Specification it is necessary carefully to select R, R<sub>1</sub> and R<sub>2</sub> in the ester in conventional manner so that the fluid has the desired physical properties and meets the rubber swell requirement of the specification. While in some cases it may be possible to use one of the foregoing esters by itself, or a mixture of two or more such esters it will usually be necessary to modify the action of the ester or esters on rubber

by incorporating a minor proportion of one or more polyoxyglycol ethers. The addition of such polyoxyglycol ethers also improves the water tolerance of the fluid which is one of the requirements of SAE 70R3 specification. Thus, for example, di(methyl oxitol) succinate by itself failed the water tolerance test at -40° C., but this difficulty was overcome by incorporating 10 percent of mixed polyoxyethylene glycol ethers. This water tolerance test is carried out by adding 3.5 percent of water to the composition and holding it at -40° C. for 24 hours; no ice formation or cloudiness must occur.

The invention also provides a hydraulic system containing a hydraulic fluid consisting of, or comprising a major proportion, preferably at least 80 percent of at least one ester having the general formula:



where R, R<sup>1</sup>, R<sup>2</sup> and n are as defined above. Additives as described above may be included in minor proportions in the fluid. Alternatively the fluid may consist entirely of one or

25 more of the esters with no additons. The invention also includes a method of operating a hydraulic system which method comprises employing a hydraulic fluid consisting of, or comprising a major proportion, preferably at least 80 percent, of the ester defined above.

30 The effect on rubber of typical esters of the present invention is shown in tables II and III. The results given in table II were those obtained when a piece of a natural rubber of the type normally used in hydraulic and brake systems was immersed in the fluid under test at 70° C. The percentage volume

35 swell was determined by using the Archimedean principle, the rubber being weighed while suspended in water before and after test. Results of similar tests carried out using a synthetic rubber of the type normally used in hydraulic systems are given in table III. In the case of natural rubber no particular limit is set but the normally accepted maximum is 5 percent and in the case of synthetic rubber the upper limit set by some manufacturers of brake systems is 15 percent. In both cases the rubber should not be unduly dry and should not be cracked or unduly soft. All the esters shown were satisfactory

40 in this respect.

45 The following examples illustrate typical hydraulic fluid compositions in accordance with the present invention:

#### EXAMPLE 1

50 99 percent Di(methyl oxitol) succinate  
 1 percent Primene 81-R (Reg. Trade Mark for a tertiary alkyl primary amine having 12 to 14 carbon atoms).  
 This composition had viscosities of 1,680 cS. at -40° C.,  
 55 3.75 cS. at 50° C. and 1.59 cS. at 100° C., and a boiling point of 292° C.

60 This composition, although representing a useful brake fluid, failed the SAE 70R3 Specification in respect of the -40° C. water tolerance clarity clause.

#### EXAMPLE 2

65 87.9 percent Di(methyl oxitol) succinate  
 10 percent Mixed polyoxyethylene glycol ethers  
 1 percent Ucon 50 HB 5100  
 0.1 percent Benzotriazole  
 1 percent Primene 81R  
 This composition had viscosities of 1,640 cS. at -40° C. 4.2 cS. at 50° C. and 1.68 cS. at 100° C. and in initial boiling point of 282° C. It also passed the SAE 70R3 water tolerance and low temperature requirements.

70 In this blend the object of the Ucon 50HB 5100, a polyoxyethylene polyoxypropylene glycol ether, was to increase the viscosity, while the benzotriazole was to inhibit corrosion of copper. The amine was present to raise the pH in accordance with the SAE 70R3 limits.

In two laboratory hygroscopicity tests carried out at different times, as previously described, 150ml. samples of hydraulic fluids were placed in open 250 ml. beakers and exposed to the atmosphere of the laboratory for 3 to 6 days. Boiling points were measured before and after exposure. Fluids A and B are the typical prior art fluids discussed in the preamble. The following results were obtained

## BOILING POINT °C.

|           | Initial | After<br>3 days | After<br>6 days |
|-----------|---------|-----------------|-----------------|
| Fluid A:  |         |                 |                 |
| 1st test  | 223     | —               | 130             |
| 2nd test  | 210     | 134             | —               |
| Fluid B:  |         |                 |                 |
| 1st test  | 271     | —               | 147             |
| 2nd test  | 272     | 147             | —               |
| Example 1 | 292     | —               | 210             |
| Example 2 | 282     | 202             | —               |

The excellent low-hygroscopicities of the fluids of this invention are further demonstrated with reference to examples 3-8 in table IV, a direct comparison having been made with fluid B of the prior art.

Two further examples of corrosion-inhibited compositions are given below (example 9 and 10)

## EXAMPLE 9

25 percent Di(methyl trioxitol) adipate  
60 percent Di(methyl oxitol) nylonate  
14 percent Ucon 50 HB 55  
1 percent Reoplex 400  
0.5 percent Di-n-butylamine  
0.1 percent Benzotriazole

20

15

25

30

35

## EXAMPLE 10

40 percent Di(methyl trioxitol) adipate  
53.9 percent Di(methyl oxitol) adipate  
5 percent Ucon H.436  
0.5 percent Di-n-butylamine  
0.5 percent Phenyl- $\alpha$ -naphthylamine  
0.1 percent Benzotriazole

The blends of examples 9 and 10 were subjected to the full test laid out in the S.A.E. 70R3 specification as drawn up by the Society of Automotive Engineers.

The fluids were entirely satisfactory apart from the boiling point change and the pH after corrosion. However these results were not considered to be detrimental in view of the fact that the boiling point after test was far in excess of that of any current fluid and the pH after corrosion was irrelevant provided that the corrosion test was satisfactory in other respects.

## EXAMPLE 11

39.9 percent Di(methyl trioxitol) adipate  
53.9 percent Di(methyl oxitol) adipate  
5 percent Ucon H 436  
0.5 percent Di-n-butylamine  
0.5 Phenyl- $\beta$ -naphthylamine  
0.1 percent Benzotriazole  
0.1 percent Phenothiazine

This fluid, which is very similar to that of example 10, passed all the tests of the S.A.E. 70R3 Specification. The phenothiazine appeared to act in controlling the pH, and in further reducing corrosion.

The hydraulic fluids of this invention as described in the examples are suitable for use under high temperature conditions, have relatively low hygroscopicity and retain high boiling points over extended periods of use.

TABLE I

| Ester                           | Viscosities cS at |       |       | SAE 70R3<br>Boiling<br>Point °C |
|---------------------------------|-------------------|-------|-------|---------------------------------|
|                                 | -40°C.            | 38°C. | 99°C. |                                 |
| Di (methyl oxitol) Succinate    | 1565              | 5.26  | 1.55  | 293                             |
| Di (methyl dioxitol) Succinate  | 8310              | 10.8  | 2.56  | 298                             |
| Di (methyl trioxitol) Succinate | Too thick         | 24.25 | 4.63  | 303                             |
| Di (ethyl oxitol) Succinate     | 1870              | 5.33  | 1.59  | 287                             |
| Di (ethyl dioxitol) Succinate   | 14,510            | 11.22 | 2.69  | 277                             |
| Di (ethyl trioxitol) Succinate  | Too thick         | 18.65 | 4.06  | 321                             |
| Di (methyl oxitol) Adipate      | 534               | 5.63  | 1.76  | 293                             |
| Di (methyl dioxitol) Adipate    | 2005              | 9.78  | 2.73  | 308                             |
| Di (methyl trioxitol) Adipate   | 11,000            | 13.89 | 3.43  | 309                             |
| Di (ethyl oxitol) Adipate       | 696.3             | 5.95  | 1.83  | 316                             |
| Di (ethyl dioxitol) Adipate     | 2458              | 9.94  | 2.70  | 316                             |
| Di (ethyl trioxitol) Adipate    | 11,704            | 17.95 | 2.95  | 316                             |
| Di (methyl oxitol) Sebacate     | solid             | 8.26  | 2.38  | 321                             |
| Di (methyl dioxitol) Sebacate   | solid             | 14.43 | 3.69  | 302                             |
| Di (methyl trioxitol) Sebacate  | solid             | 26.00 | 5.89  | 307                             |
| Di (ethyl oxitol) Sebacate      | solid             | 8.73  | 2.55  | 340                             |
| Di (ethyl dioxitol) Sebacate    | solid             | 10.35 | 4.03  | 314                             |
| Di (ethyl trioxitol) Sebacate   | solid             | 27.00 | 5.94  | 316                             |
| Di (methyl oxitol) Azelate      | 812               | 8.27  | 2.38  | 336                             |
| Di (methyl dioxitol) Azelate    | 2490              | 12.99 | 3.39  | 310                             |
| Di (methyl trioxitol) Azelate   | 9,660             | 24.51 | 5.58  | 318                             |
| Di (ethyl oxitol) Azelate       | solid             | 8.44  | 2.75  | 333                             |
| Di (ethyl dioxitol) Azelate     | 2135              | 11.78 | 3.18  | 284                             |
| Di (ethyl trioxitol) Azelate    | 6824              | 19.73 | 4.75  | 298                             |
| +Di (methyl oxitol) Nylonate    | 647               | 5.23  | 1.67  | 282                             |

+An ester prepared by reacting ethylene glycol mono methyl ether with a mixture known as "A.G.S. Acid" and containing approximately 15.25% adipic acid, 1% glutaric acid and 25.35% succinic acid. The material is supplied by Imperial Chemical Industries Limited.

TABLE II

| Fluid                         | % Volume Increase on Natural Rubber at 70° C. |        |
|-------------------------------|-----------------------------------------------|--------|
|                               | 2 days                                        | 1 week |
| Di(methyl oxitol) Succinate   | 2.36                                          | 1.26   |
| Di(methyl dioxitol) Succinate | -3.98                                         | 2.53   |
| Di(ethyl trioxitol) Succinate | 0.23                                          | 0.39   |
| Di(methyl oxitol) Adipate     | 4.39                                          | 3.77   |
| Di(methyl trioxitol) Adipate  | -0.31                                         | -1.53  |
| Di(ethyl trioxitol) Adipate   | 1.17                                          | 2.82   |
| Di(methyl trioxitol) Azelate  | 1.32                                          | 1.22   |
| Di(methyl oxitol) Nylonate    | 2.71                                          | 2.21   |

TABLE III

| Ester                          | % Volume increase synthetic rubber 3 days at 120° C. |    |
|--------------------------------|------------------------------------------------------|----|
|                                | 20                                                   | 25 |
| Di(methyl dioxitol) Succinate  | 7.48                                                 |    |
| Di(methyl trioxitol) Succinate | 4.72                                                 |    |
| Di(methyl trioxitol) Adipate   | 2.44                                                 |    |
| Di(ethyl oxitol) Adipate       | 8.52                                                 |    |
| Di(ethyl dioxitol) Adipate     | 14.1                                                 |    |
| Di(ethyl trioxitol) Adipate    | 12.9                                                 |    |
| Di(methyl trioxitol) Sebacate  | 8.6                                                  |    |
| Di(methyl trioxitol) Azelate   | 2.65                                                 |    |
| Di(ethyl trioxitol) Azelate    | 7.62                                                 |    |
| +Di(methyl oxitol) Nylonate    | 13.20                                                |    |

+An ester prepared by reacting ethylene glycol mono methyl ether with a mixture known as "A.G.S. Acid" and containing approximately 15-25 percent adipic acid, 45-60 percent glutaric acid and 25-35 percent succinic acid.

TABLE IV

Hygroscopicity Tests

| Ex. No. | Blend                                                              | Percent humidity in the above four tests | Boiling point ° C. at— |       | Boiling point ° C. after— |        |        |        |
|---------|--------------------------------------------------------------------|------------------------------------------|------------------------|-------|---------------------------|--------|--------|--------|
|         |                                                                    |                                          | Initial                | 1 day | 2 days                    | 3 days | 4 days | 5 days |
| 3.....  | 80% di(methyl oxitol) nylonate; 20% special castor                 |                                          | 294                    | 284   | 239                       | 221    | .....  | 186    |
| 4.....  | 80% di(methyl oxitol) succinate; 20% special castor                |                                          | 292                    | 270   | 242                       | 216    | .....  | 187    |
| 5.....  | 80% di(methyl oxitol) adipate; 20% special castor                  |                                          | 297                    | 287   | 234                       | 210    | .....  | 184    |
|         | Fluid B                                                            |                                          | 268                    | 221   | 161                       | 146    | .....  | 126    |
|         |                                                                    |                                          | 48.5                   | 46    | 61.5                      | 61.0   | .....  | 65     |
| 6.....  | 8% MB castor; 12% special castor; 80% di(methyl oxitol) nylonate   |                                          | 279                    | 238   | 221                       | .....  | 201    |        |
| 7.....  | 5% Ucon 50HB 5,100; 2% Reoplex 400; 93% di(methyl oxitol) nylonate |                                          | 280                    | 264   | 232                       | .....  | 204    |        |
| 8.....  | 4% Reoplex 400; 96% di(methyl oxitol) nylonate                     |                                          | 282                    | 249   | 227                       | .....  | 205    |        |
|         | Fluid B                                                            |                                          | 268                    | 209   | 182                       | .....  | 148    |        |

## NOTE:

The Special Castor was an ethylene oxide/propylene oxide treated castor.

MB castor is a heat treated air blown castor oil.

Reoplex 400 was a polyoxyethylene glycol adipate of molecular weight 400 marketed by Geigy Ltd.

Ucon 50HB 5,100 was a polyoxyethylene polyoxypropylene glycol ether marketed by Union Carbide and having a viscosity of about 5,100 S.U.S. at 100° F.

## We claim:

1. In a method of hydraulic transmission of power to pressure operated elements the improvement which comprises employing as the hydraulic fluid a composition consisting essentially of a mixture of the following components:

a. an ester or mixture of esters of the formula

where R is an alkylene group of two to eight carbon atoms, R<sup>1</sup> is selected from the group consisting of an alkyl radical of one to four carbon atoms and a phenyl radical, R<sup>2</sup> is selected from the group consisting of ethylene, propylene and butylene, and n is an integer of from 0 to 3; and b. an organic antioxidant;

said component (a) being present in the mixture in an amount of at least 50 percent by weight based on the total weight of the mixture and components (a) and (b) being so selected to provide a mixture having a kinematic viscosity at -40° C. of not more than 5,000 cS. and a boiling point of at least 260° C.

2. In a method of hydraulic transmission of power to pressure operated elements the improvement which comprises employing as the hydraulic fluid a composition consisting essentially of a mixture of the following components:

a an ester or mixture of esters of the formula



where R is an alkylene group of two to eight carbon atoms.

R<sup>1</sup> is selected from the group consisting of an alkyl radical of one to four carbon atoms and a phenyl radical,

R<sup>2</sup> is selected from the group consisting of ethylene, propylene and butylene, and

n is an integer of from 0 to 3; and

b. an organic corrosion inhibitor;

said component (a) being present in the mixture in an amount of at least 50 percent by weight based on the total weight of the mixture and components (a) and (b) being so selected to provide a mixture having a kinematic

viscosity at -40° C. of not more than 5000 cS. and a boiling point of at least 260° C.

3. In a method of hydraulic transmission of power to pressure operated elements the improvement which comprises employing as the hydraulic fluid a composition consisting essentially of a mixture of the following components;

a. an ester or mixture of esters of the formula



where R is an alkylene group of two to eight carbon atoms, R<sup>1</sup> is selected from the group consisting of an alkyl radical of one to four carbon atoms and a phenyl radical, R<sup>2</sup> is selected from the group consisting of ethylene, propylene and butylene, and n is an integer of from 0 to 3; and b. a lubricity agent selected from the group consisting of castor oils, triaryl borates, triaryl phosphates, polyoxyalkylene glycols and ethers thereof, orthophosphates of primary and secondary amines, sulfates of primary and secondary amines, dialkyl citrates, saturated aliphatic dibasic carboxylic acids and alkyl esters thereof, and unsaturated aliphatic acids and their salts; said component (a) being present in the mixture in an amount of at least 50 percent weight based on the total weight of the mixture and components (a) and (b) being so selected to provide a mixture having a kinematic viscosity at -40 °C. of not more than 5000cS. and a boiling point of at least 260°C.

4. In a method of hydraulic transmission of power to pressure operated elements, the improvement comprising employing as the hydraulic fluid a mixture consisting essentially of esters of the formula



where R is an alkylene group of two to eight carbon atoms, R<sup>1</sup> is selected from the group consisting of an alkyl radical of one to four carbon atoms and a phenyl radical, R<sup>2</sup> is selected from the group consisting of ethylene, propylene and butylene, and n is an integer of from 0 to 3, said ester mixture containing a major proportion of esters prepared by reacting ethylene glycol monomethyl ether with a mixture of dibasic acids containing approximately 15-25 percent adipic acid, 45-60 percent glutaric acid and 25-35 percent succinic acid, and a minor proportion of di(triethylene glycol monomethyl ether) adipate.

5. The method of claim 3 wherein said composition includes an organic antioxidant.
6. The method of claim 3 wherein said composition includes an organic corrosion inhibitor.
7. The method of claim 3 wherein said composition includes an organic antioxidant and an organic corrosion inhibitor.
8. The method of claim 3 wherein component (b) of said composition is a polyoxyalkylene glycol or ether thereof in an amount of from about 5 percent to about 14 percent by weight of said composition.
9. The method of claim 3 wherein R<sup>1</sup> of the formula for said ester component (a) is selected from the group consisting of methyl and ethyl.
10. The method of claim 3 wherein R<sup>1</sup> is methyl.
11. The method of claim 3 wherein R<sup>2</sup> is ethylene.
12. The method of claim 3 wherein R is an alkylene group of two to four carbon atoms.
13. The method of claim 3 wherein said ester or mixture of esters is derived for an acid selected from the group consisting of succinic, glutaric, adipic, azelaic, sebacic, and isosebacic acids and mixtures thereof.
14. The method of claim 3 wherein component (a) is a mixture of esters of the recited formula, said mixture of esters being derived from a mixture of esters consisting of adipic acid, glutaric acid and succinic acid.
15. The method of claim 14 wherein the mixture of acids consists of approximately 15 to 25 adipic acid, 45 to 60 percent glutaric acid and 25 to 35 percent succinic acid.
16. The method of claim 3 wherein the component (a) derived from a glycol ether selected from the group consisting of methyl and ethyl ethers of mono-, di-, and triethylene glycols.
17. The method of claim 3 wherein said component (a) comprises a mixture of esters prepared by reacting ethylene glycol monomethyl ether with a mixture of dibasic acids consisting of 15 to 25 percent adipic acid, 45 to 60 percent glutaric acid, and 25 to 35 percent succinic acid.
18. The method of claim 17 wherein said component (a) additionally comprises di(triethylene glycol monomethyl ether) adipate.
19. The method of claim 3 wherein said component (a) is present in the mixture in an amount of at least 80 percent by weight based on the total weight of the mixture.

\* \* \* \* \*